

# UNITED STATES PATENT OFFICE.

AUGUSTE J. ROSSI AND LOUIS E. BARTON, OF NIAGARA FALLS, NEW YORK, ASSIGNEES TO THE TITANIUM ALLOY MANUFACTURING COMPANY, OF NEW YORK, N. Y., A CORPORATION OF MAINE.

## METHOD FOR CONCENTRATING TITANIC OXID FROM SUBSTANCES CONTAINING IT AND IRON OXID.

1,106,408.

Specification of Letters Patent.

Patented Aug. 11, 1914.

No Drawing.

Application filed November 29, 1912. Serial No. 733,945.

To all whom it may concern:

Be it known that we, AUGUSTE J. ROSSI and LOUIS E. BARTON, both citizens of the United States, and residents of Niagara Falls, in the county of Niagara and State of New York, have jointly invented certain new and useful Improvements in Methods for Concentrating Titanic Oxid from Substances Containing It and Iron Oxid, of which the following is a specification.

Uses of titanic oxid in the arts are now extensive and increasing. A long standing problem has been, and still is, its accumulation, on industrial scales of manufacture, in sufficient quantity and purity, and at the least possible cost.

Numerous known substances contain greater or less percentages of titanic oxid ( $TiO_2$ ). Natural titanic oxid is, as well known, widely and plentifully existant in ores, but, almost invariably, so entangled, or combined, with other oxids, and constituents of the gangue, as to render it, as mined, unavailable for most industrial purposes. As thus found, in varying percentages, in enormous existing deposits of so-called "titaniferous-iron," or "ilmeno-rutile," ores, it is particularly associated with corresponding percentages of iron oxids, from which it has hitherto proved practically impossible, without prohibitory expense, to so completely separate it as to render it available for many desired industrial uses. Even the purest of such ores, being those commonly called "rutile," ores, though of much higher titanic oxid content than any others, as high for example as 95%, contain nevertheless percentages of iron oxids, silica and earthy bases, such as alumina, rendering them, in natural state, unsatisfactory contributors of titanic oxid in the manufacture of certain special products, and, moreover, deposits of such "rutile" ores have hitherto been discovered only in segregated quantities too small to supply existing industrial demand. Moreover the said ores usually contain more or less "ilmenite" being a compound of titanic oxid and iron oxid designated by the formulas  $FeTiO_3$  or  $FeOTiO_2$ , which compounds we believe to have hitherto proved too refractory for any commercially practicable method of deriving titanic oxid from such last mentioned ores.

The objects of our present invention comprise production of methods whereby titanic oxid may be more completely separated from the other, and particularly the iron, constituents of said ores, and this more rapidly, simply, and economically, and with a better resultant titanic oxid product than heretofore. We attain these objects by our present improved method as follows:—We first finely pulverize the ore and thoroughly mix the resulting powder with hydroxid of an alkali metal, preferably caustic soda, *i. e.* sodium hydroxid ( $NaOH$ ). The proportion of soda thus employed as such should be amply sufficient to enable it to fully react, during our next step, with all constituents of the ore having chemical affinity therefor. Excess of soda above this is neither injurious, nor prohibitarily expensive for reasons hereinafter stated. For example, in treating an ore which analyzed

|              |    |    |
|--------------|----|----|
| Titanic oxid | 52 | 75 |
| Iron oxids   | 40 |    |
| Silica       | 3  |    |
| Alumina      | 4  |    |

we obtained excellent results by adding the soda in a proportion of 58 parts (of a 70%  $Na_2O$  commercial caustic soda) to each 100 parts of ore, as we prefer that the proportion of soda added should be sufficient to insure formation during our next step of sodium titanate ( $Na_2TiO_3$ ), but we do not limit ourselves to such proportion, having attained by our process good results with considerably less soda. Our next step is to thoroughly melt our said mixture of ore and sodium hydroxid. The melting operation is preferably conducted in an electric furnace, but it may of course be accomplished by any other means capable of insuring a thorough and complete melt, as for example in an open hearth furnace heated by a direct coke fire in a grate, or indirectly by producer gas, such furnaces being of course lined with material sufficiently refractory to resist the action of the charge during the melt. During the latter we believe that the following reactions, among others, occur in the charge, *viz*:—Oxid of sodium combines with oxid of titanium to form titanate of soda, thus readily breaking up the said ilmenite molecules present and releasing in a state after-

ward soluble, as hereinafter described, iron 5  
oxid constituents. Ferrous oxid of iron is  
more or less oxidized to ferric oxid. Silica  
and alumina of the gangue combine with the  
oxid of sodium to form silicates and alumini-  
nates of soda. The melt is then cooled and  
well crushed,—say to about 80 mesh. It is  
then repeatedly and thoroughly lixiviated in  
heated, preferably boiling, water, until sub-  
stantially all of said titanate of soda has  
10 been decomposed into titanic oxide and  
caustic soda. The soda thus set free, also  
any excess soda, and said silicates and alumini-  
nates, etc., being soluble, dissolve and are thus  
15 removed from the remaining melt with the  
water of lixiviation. The soda lye resulting  
from said lixiviation may be evaporated to  
a cake of soda useful in treating as afore-  
said the next charge of ore. In our practice  
20 we have thus repeatedly recuperated from  
85% to 90% of the soda employed, the which  
constitutes a notable economy of our present  
method. What remains undissolved of the  
melt during its aforesaid lixiviation is sepa-  
25 rated, as by decantation, and may be ex-  
pected to be substantially free from excess  
of soda and from silica and alumina and  
their compounds, but to retain substantially  
30 all of the titanic oxide and iron oxids, the  
which are insoluble in water, and also some  
slight remainders of gangue including mag-  
nesia, the ores referred to containing not to  
substantially exceed traces of lime. The  
35 said remainder of the melt we then treat, pref-  
erably while still moist, to a heated, prefer-  
ably boiling, bath containing acid so dilute  
as to dissolve therein iron, rather than tit-  
anium, compounds, preferably sulfuric acid,  
40 owing to the latter's comparative cheapness,  
and superior results, though other suitable  
acids, such as hydrochloric for example, may  
be employed. In this step of our method we  
have, with excellent results, proportioned the  
45 water of the bath to be from three to four  
times the weight of the therein boiled melt,  
and the acid, for example sulfuric acid, in  
proportion of from about twenty-nine parts  
to each twenty parts of said remainder of  
50 the melt. Though, by these proportions, the  
sulfuric acid is in considerable excess, it is  
not wasted, since it may be withdrawn, or  
decanted, to be used, with or without addi-  
tion of fresh acid, in treatment of the next  
55 charge. This last mentioned treatment of  
the melt we continue for about an hour, after  
which the titanic acid, the which remains in  
the bath undissolved, will settle to the bot-  
tom, and, being separated, as by decantation,  
60 these settling will, if our method has been  
properly followed as above, be found, after  
calcining them, to consist of pure titanic  
oxid in proportion as high as from 94% to  
96%. We are thus enabled to produce from  
65 ordinary titaniferous-iron, or ilmeno-rutile,  
ores, and, as we believe, by a more rapid,

simple, and economical process than hereto-  
fore, a titanic oxid product higher in its  
percentage of that compound than the best  
and rarest rutile ores, and this at a cost very  
greatly below the present market price of  
70 such last mentioned ores. Moreover by re-  
peating our said process on our said product  
it may thereby, the same as may such rutile  
ores, be readily, and economically, brought  
75 to contain still higher percentages of pure  
titanic oxid.

We are aware that heretofore it has been  
directed that, as a step in desired production  
of soluble compounds of titanium, as dis-  
tinguished from titanic oxid, certain ma-  
terials containing the latter, as for example  
banxite, or even rutile or ilmenite previously  
fused with carbonate of soda, be fluxed with  
acid sodium sulfate or sodium pyrosulfate  
for the express purpose of dissolving out or  
80 rendering soluble the titanic oxid contained  
in such materials, after which the resulting  
melt is directed to be treated with dilute  
sulfuric acid maintained however so acidified  
85 as to prevent the titanic oxid from pre-  
cipitating out of its said solution. We do  
not of course claim any such procedures, the  
which in operation and results are obviously  
the reverse of our own, it being observed  
90 that in our aforesaid method the conditions  
are such that the natural titanic oxid is  
throughout prevented from dissolving or  
forming other compounds requiring hereto-  
fore necessitated protracted and expensive  
95 boiling or other treatment to insure its pre-  
cipitation and separation from the bath.  
We believe ourselves to be the first to flux  
100 the raw titaniferous material with hydroxid  
of an alkaline metal, thereby breaking up  
the ilmenite molecules, and also thereby  
105 forming titanates, substantially all of which  
latter, during our lixiviation in water, part  
with their soluble soda, while substantially  
110 all of the thus liberated titanic oxid being  
insoluble, under the conditions of said dilute  
acid bath, settles immediately therein as  
115 such, or more or less hydrated, without dis-  
solving, whereby iron oxids present are sepa-  
rated therefrom because, under said condi-  
tions, reacting to form sulfates which re-  
main in solution in said bath. We are also  
120 aware that it has been asserted, prior to our  
invention, that titanic acid may be obtained  
from suitable bauxite containing a percent-  
age thereof besides alumina, silica and ferric  
125 oxid, by stirring the same into sulfuric acid  
of 100 degrees Tw., the solution being after-  
ward diluted to 60 degrees Tw., and boiled  
until the dissolved titanic acid precipitates,  
but this again is not our process for the  
130 reasons aforesaid, it being borne in mind  
that the latter avoids substantially entirely  
such previous productions of acid, soluble,  
compounds of titanic acid as preliminary  
steps, that our process is aimed at, in no

stage thereof, dissolving the titanic oxid, and that thereby we are enabled to separate it in mass from natural ores containing iron oxid, and at much less expenditure of reagents, time, labor, heat, etc., than has, we believe, been heretofore possible, at least when operating on industrial scales. Besides which we obtain more directly a more natural, purer, and we believe therefore, for many purposes, more efficient titanic oxid product.

It will be noted that caustic potash, (*i. e.* potassium hydroxid, KOH), can be used in the same way, and with like effect, as caustic soda, in the practice of our invention; in fact the hydroxid of any alkaline metal may, if desired, be so substituted for sodium hydroxid. It will however be appreciated that the latter is economically, and therefore industrially, more desirable so long as present comparative market prices of these respective oxids are maintained, and moreover we also prefer the latter because of its superior action and effect in the practice of our said method.

It will be understood that carbonate of soda might, though with inferior results and at greater expense, be used as a substitute for a hydroxid of an alkali metal in the practice of our method, and this without departing from our invention, the which, in its broadest aspects, comprises the step of melting the substance containing titanic and iron oxids with oxid of an alkali metal in novel combination with our aforesaid steps of lixiviating in water the resulting melt and subjecting the remainder thereof to the action of a bath containing an acid so dilute as to dissolve therein iron, but not therein titanium, compounds, as hereinbefore described. But our researches have demonstrated that no other compounds of sodium, or alkaline compounds of soda, are capable of producing, with equal rapidity, effectiveness and completeness, the reactions required to separate the titanic from the other oxid therewith entangled as are said hydroxids of alkali metals, including particularly caustic soda, when, as per our method, charged as such in making our melt. The employment, in this connection, of even carbonate of soda we have found comparatively inefficient, inasmuch as, while this may ultimately result in production in the melt of soda to a greater or less extent, it requires, owing to its necessarily greater relative bulk, to its content of carbonic anhydrid, and to its greater stability, additional treatments, or at least expenditure of additional time and heat, to insure even its inferior performance of said required reactions, as evidenced for example by the instance hereinbefore referred to in which, owing to the aforesaid substantially prohibitory characteristics of said carbonate, the product derived from its fusion with

rutile or ilmenite is subsequently fluxed with acid sodium sulfate, etc., in order to render it available.

While we have particularly referred, throughout our preceding specification, to ores, we do not wish thereby to confine the application of our methods to ores specifically, it being understood that such application to any other suitable substance, or material, containing titanic acid and iron oxid is also feasible and within the purview of our invention and claims.

What we claim as new and desire to secure by Letters Patent is the following, viz:—

1. The method of obtaining titanic oxid ( $TiO_2$ ) from a substance containing it and iron oxid, which comprises melting said substance together with oxid of an alkali metal, lixiviating the resulting melt in hot water, withdrawing the undissolved residue of said melt and subjecting it to the action of a bath containing acid so dilute as to dissolve therein iron, rather than titanium, compounds.

2. The method of obtaining titanic oxid ( $TiO_2$ ) from a substance containing it and iron oxid, which comprises melting said substance together with hydroxid of an alkali metal charged as such, lixiviating the resulting melt in hot water, withdrawing the undissolved residue of said melt and subjecting it to the action of a bath containing sulfuric acid so dilute as to dissolve therein iron, rather than titanium, compounds.

3. The method of obtaining titanic oxid ( $TiO_2$ ) from a substance containing it and iron oxid, which comprises melting said substance together with sodium hydroxid charged as such, lixiviating the resulting melt in hot water, withdrawing the undissolved residue of said melt and subjecting it to the action of a bath containing acid so dilute as to dissolve therein iron, rather than titanium, compounds.

4. The method of obtaining titanic oxid ( $TiO_2$ ) from a substance containing it and iron oxid, which comprises melting said substance together with sodium hydroxid charged as such, lixiviating the resulting melt in hot water, withdrawing the undissolved residue of said melt and subjecting it to the action of a bath containing sulfuric acid so dilute as to dissolve therein iron, rather than titanium, compounds.

5. The method of obtaining titanic oxid ( $TiO_2$ ) from a substance containing it and iron oxid, which comprises melting said substance together with oxid of an alkali metal, lixiviating the resulting melt in hot water, withdrawing the undissolved residue of said melt, subjecting it to the action of a bath containing acid so dilute as to dissolve therein iron, rather than titanium, com-

pounds, and finally withdrawing and calcining the undissolved residue.

6. The method of obtaining titanic oxid ( $TiO_2$ ) from a substance containing it and iron oxid, which comprises melting said substance together with hydroxid of an alkali metal charged as such, lixiviating the resulting melt in hot water, withdrawing the undissolved residue of said melt and subjecting it to the action of a bath containing sulfuric acid so dilute as to dissolve therein iron, rather than titanium, compounds, and finally withdrawing and calcining the undissolved residue.
- 10 7. The method of obtaining titanic oxid ( $TiO_2$ ) from a substance containing it and iron oxid, which comprises melting said substance together with sodium hydroxid charged as such, lixiviating the resulting melt in hot water, withdrawing the undissolved residue of said melt and subjecting
- 15
- 20

it to the action of a bath containing acid so dilute as to dissolve therein iron, rather than titanium, compounds, and finally withdrawing and calcining the undissolved residue.

25

8. The method of obtaining titanic oxid ( $TiO_2$ ) from a substance containing it and iron oxid, which comprises melting said substance together with sodium hydroxid charged as such, lixiviating the resulting melt in hot water, withdrawing the undissolved residue of said melt and subjecting it to the action of a bath containing sulfuric acid so dilute as to dissolve therein iron, rather than titanium, compounds, and finally withdrawing and calcining the undissolved residue.

30

35

AUGUSTE J. ROSSI.  
LOUIS E. BARTON.

Witnesses:

WALTER D. EDMONDS,  
PHILIP C. PECK.